

O. C. WINESTOCK.  
DEINKING PROCESS.  
APPLICATION FILED MAY 29, 1912.

1,138,596.

Patented May 4, 1915.



## Witnesses

Witnesses  
J. P. Gormley  
J. R. Willow.

OTTO C. WINESTOCK  
Inventor  
by *Cadman & Co.* Attorneys

# UNITED STATES PATENT OFFICE.

OTTO CHARLES WINESTOCK, OF PERKINSVILLE, VERMONT, ASSIGNOR TO THE GENERAL WASTE-PAPER RECOVERY COMPANY, OF BALTIMORE, MARYLAND, A CORPORATION OF DELAWARE.

## DEINKING PROCESS.

1,138,596.

Specification of Letters Patent.

Patented May 4, 1915.

Application filed May 29, 1912. Serial No. 700,547.

To all whom it may concern:

Be it known that I, OTTO C. WINESTOCK, a citizen of the United States, residing at Perkinsville, in the county of Windsor and 5 State of Vermont, have invented a new and useful Deinking Process, of which the following is a specification.

This invention relates to a process for defibering either printed or unprinted paper 10 and for removing the ink from print paper.

The general principle of my process of deinking and de-fibering printed paper will be understood from the following description.

15 The desideratum in this art is to reduce the printed paper to an ink-free pulp without shortening, weakening or discoloring the fibers which were felted together to form the original paper. The approximate fulfilment 20 of these conditions requires that the fibers be disentangled or de-felted with the minimum amount of cutting or breakage, and that the removal of the ink be accomplished without exposing the paper to such prolonged boiling or soaking in strong alkali 25 or other material as will rot or weaken or discolor the fiber. In searching for a process and means for carrying it out which shall approximately meet the above conditions, I 30 have found that certain principles hitherto undiscovered, are essential and constitute the necessary basis for success. These will first be stated broadly and afterward I will 35 specify in detail the exact conditions and apparatus with which I have achieved the greatest measure of success.

I have found that when wet paper printed in ordinary black ink is torn, any ink which is on the line of tear is much loosened by the 40 pulling apart of the paper fibers, so that the adhesion of such portions of the ink as remain on the fringe of disengaged fibers at the torn edge is much less than the normal adhesion of ink to un torn paper, and it became my aim to find a cheap and practical 45 mechanical method of shredding or tearing the paper into such fine bits that the paper-fiber foundation to which each particle of ink adhered would be wholly or partly 50 pulled apart, thus putting the ink in condition for easy removal by a simultaneous or even a subsequent treatment much less prolonged and severe than would be necessary if this foundation were undisturbed. The 55 ideal accomplishment of this aim requires

nearly complete defelting or disentangling of the fibers of the paper; and while I recognized at first that it might not be possible to fully realize this ideal I have worked toward it and found that the means herein described 60 and specified and forming the subject of my co-pending apparatus application Serial No. 700,546, filed May 29, 1912, accomplished it to a surprisingly complete extent. I have found that the best results are achieved by 65 treating the paper during the time of defelting or disintegration with the chemical agents, or detergents, adapted to further loosen and to carry away the ink rather than by so treating it subsequently. It will be 70 seen in the detailed description of my apparatus that the loosening action on the ink due to pulling the fibers apart is aided by mechanical attrition by the machine which tends further to mechanically remove the 75 ink, and this doubtless accounts in some measure for the better results achieved when the detergent is present during the process of defibering so that full advantage is taken of this mechanical attrition. I have found 80 that a relatively mild chemical agent and a temperature only moderately high is all that is necessary for accomplishing the removal of the ink when used in this way. The detergent which I use is in general a soap 85 containing some sodium silicate and preferably some free alkali.

The requirements for tearing paper, crudely stated, are that the paper should be held at two or more places and pulled 90 apart. So long as the paper is not reduced to pieces below a certain size, this is extremely easy by the use of mechanical expedients which readily suggest themselves but when it becomes necessary to approximate at all closely the above defined ideal 95 conditions which I have set out to fulfil, the difficulties materially increase. It is of course possible to accomplish the defibering in the well known beating engine or jordan, 100 but I have found that these or equivalent devices not only require very many times as long as does my apparatus, but also tend to grind the ink into the fiber of the paper so that the loosening action, due to tearing and 105 defibering is almost wholly nullified and offset. There is also always a tendency in these machines to cut and shorten the fiber. Some of the so-called digesters used in the 110 art do not employ such close contact be-

5 between the moving and stationary mechanical members as that in beaters and jordans and these are therefore not open to the same objection of pounding or pressing the partly loosened ink particles back into intimate contact with the fiber, but on the other hand they do not reduce the average size of torn particles to anything approaching the smallness which is desired, and in consequence 10 relatively large portions of ink still remain on an unshaken and undisturbed mat of fibers and require for their removal the same drastic chemical processes that are required for larger pieces of paper.

15 In my apparatus I have abandoned the idea of holding the paper mechanically in the ordinary sense of the word, and I depend upon the principle which I believe to be broadly new in this art, of holding the 20 paper while it is torn or shredded, through dependence upon its inertia, aided by the inertia of a fluid medium such as a liquid with which it is surrounded and in which it is suspended.

25 It is of course recognized that the degree in which mechanical strength and inertia contribute toward the resistance of a body to force applied to it is a function of the 30 time available in which it may respond to this force. In conformity with this general law of physics, I find that a slow moving blade or equivalent striking upon a piece of paper invested or embedded, so to speak, in a liquid, will tear that paper only if the size 35 of the piece is relatively large, while if the piece is relatively small it will take up the motion of the blade or else be brushed or swept aside by it without being torn or perceptibly strained; that as the relative 40 speed of the blade increases, the minimum piece that it will tear becomes of less and less size; and, finally that if the speed is very high a very small piece of paper is unable to take up this speed soon enough to 45 avoid being torn apart. I have found that speed can, within practicable limits, be carried to such a point that a piece of paper consisting of only a few fibers felted together, held or restrained but backed by the 50 inertia of the liquid in which it is immersed, can be successfully torn apart and reduced to a condition so near that of its component single fibers as to meet very closely the criterion for ideal results which I have laid 55 down in a paragraph above. It would indeed be theoretically possible to get a speed of blade and a sharpness of edge so great that a single component fiber floating alone would be divided, but this is obviously carrying the principle to an undesirable extent. 60 The action upon the material is in the nature of a pull or strain due to opposed tendencies or influences, and these opposing tendencies or influences or conditions I have 65 for convenience termed "forces" serving to

pull apart the fiber of the material under a strain insufficient, by reason of the yielding character of one of them to cause the breakage of the fibers themselves. It became evident to me that this principle could be embodied in any of a great many ways and that different detailed embodiments would probably be required for the best solution of different detailed problems of defibering. The embodiment with which I have achieved 70 the best results is the following, which will become clear by a reference to the figures and drawings forming a part of this specification.

75 Referring to the accompanying drawing,—Figure 1 is a vertical section through my apparatus. Fig. 2 is a vertical section on the line 2—2 of Fig. 1.

The machine is suitably supported upon legs or standards 1. The paper to be defibered and de-inked is introduced into the machine through an entrance opening 2 provided with a cover 3. The opening 2 communicates with a supply chamber 4 which preferably is tapered toward its lower end, 80 as indicated at 5, and communicates with one end of a horizontally extending pipe or draft-tube 6. Communicating with the opposite end of the draft-tube 6 is an upwardly extending pipe or return passage 7 which is 85 gradually flared or increased in size in an upward direction. The pipe or return passage 7 at its upper end is continued horizontally as shown at 8 and extends into the supply chamber 4, and has its discharge end 90 directed downwardly. The direction of flow of material through the machine is indicated by the arrows.

95 Extending axially through the draft-tube 6 is an overdriven propeller shaft 9 mounted in suitable bearings 10, and having fixed thereto, within the pipe 6, one or more propellers or agitating elements 11—12. The shaft 9, on its outer end, is provided with a belt wheel or other driving means 13 capable 100 of attaining great velocity. In the machine illustrated, the propeller blade 11 is 5½ inches in diameter and the second propeller 12 located about 13 inches away from the propeller 11, is about 6½ inches in diameter. 105 The draft-tube 6 is about 7 inches in diameter. It will be understood that all of these dimensions may be increased or altered within broad limits in making a machine of a larger size than that heretofore employed 110 by me.

115 The propellers are preferably driven at so high a rate of speed that "cavitation" occurs; that is to say, the propellers revolve in a cavity of their own making. Under 120 these conditions, the leading edges of the propeller may be conceived of as continually shaving off elements of the water presented to them and throwing it with some violence 125 forward in the direction of the flow. This 130

condition seems to realize the intent of the invention better than anything else that I have thus far tried. The water, as presented to the propeller, contains the floating or suspended particles or pieces of paper which are to be defibered, defelted or reduced to pulp, and the rapidly moving blades strike these suspended particles of paper with such quickness that, embedded as they are in the water, they are unable to take up bodily the rapid motion of the propeller blades, and therefore the fibers, which may be conceived of as engaging with the edges of the propeller, are pulled out, thus defibering the paper without materially shortening the fiber while at the same time, loosening the ink as before explained. The propeller subserves the secondary function of producing rapid circulation of the material without the necessity of using a pump or other auxiliary means for this purpose.

I prefer to rotate the propellers at around 1800 to 2500 revolutions per minute. It will be observed that the mixture of water and pulp, after being cavitated by the propellers, rapidly traverses the return passage 7-8 and is discharged into the supply chamber 4, from which it passes down again to the suction side of the overdriven propellers. The speed of rotation of the water and stock in the machine is very rapid, approximating 1200 feet per minute. It will be observed that the water and stock are carried through the propellers and cavitated time and time again at an exceedingly high rate of speed.

Actual tests have demonstrated that the machine illustrated, operating on the inertia and cavitating principle, is very well suited to the purpose of carrying out the process of this invention, and that it will completely defiber the stock and deterge the ink in a period of from approximately 1½ to 10 minutes, according to the character of the paper acted upon.

In addition to the defelting action which takes place at the face of the propellers of my machine by the opposed action of the propellers and the inertia of the stock and liquid, I believe that further defelting action is due to the velocity at which the stock is thrown through the cavities produced by the propellers. The hydrodynamic action of the liquid and stock as it strikes the corners of and is driven through the return tubes 7 and 8 also has a defelting action, due I believe to the fact that the fibers on the outside of the moving mass of water and stock are retarded by frictional contact with the walls of the return tubes, while the fibers at the center pass on more rapidly. The waterfall effect at the discharge end of the tube 8 also has a separating or defelting effect.

In carrying out the process on a commercial scale, larger machines than that hereto-

fore employed by me will be used, and some of the proportions may be varied within broad limits.

In carrying out my process with so-called book paper or old magazines in a machine, such as is shown in the accompanying drawing, I prefer to use about 15 pounds of papers, which are torn up by hand into pieces several inches square. This paper is placed in any suitable charging tank filled with water of a temperature, preferably of approximately 160° F., and is permitted to remain there until the de-fibering machine is ready to receive it, after which the water and paper in the charging tank are dumped into the chamber 4 of the de-fibering machine. I prefer to permit the paper to remain in the hot water in the charging tank for from 5 to 10 minutes, but this operation can be varied. Any desired quantity of warm water can be used in the charging tank, so that the paper will be softened thereby. If a relatively small quantity of water is used in the charging tank, a proper amount of water may be put into the de-fibering machine, so that when the softened paper is fed to the de-fibering machine, the proportion of paper or pulp to the water will be approximately 15 pounds of paper to about 38 gallons of water, which corresponds to about 20 pounds of water to about one pound of dry paper, although it will be understood that these proportions can be widely varied. The water in the de-fibering machine is preferably heated to a temperature of approximately 160° F. This temperature seems to produce the best results, but can be varied. After the de-fibering machine has been charged with the water and paper or pulp, as before described, the deterging compound is added. This compound is described fully hereinafter. After charging the machine, as above described, the blades or propellers are operated preferably at about 1800 to 2500 revolutions per minute. I have found in practice that the usual time for reducing ordinary magazine paper is approximately three minutes, the water and pulp repeatedly circulating through the machine at a speed of approximately 1200 feet per minute. As before stated, with some kinds of paper, such as newspaper, the operation consumes less time and with other types of paper it may consume more. At the end of the operation the machine is stopped and the water and stock are drawn off through the outlet 15 at the bottom and placed in an ordinary paper making beater where the pulp is washed, in either hot or cold water, as desired, by means of a washing cylinder for two or three hours for the removal of the loosened ink and other foreign matter. After washing the stock, as above described, the process of defibering and deinking is completed. The

100

90

95

100

105

110

115

120

125

130

stock may then, if desired, be run through a Jordan machine to brush it out and may then be conducted to the stuff chest and on to the paper machine.

5 I have made an excellent quality of book paper from my recovered pulp without the addition of any new stock, although in paper making practice, it may sometimes be desirable to add a small percentage of new stock.

10 In carrying out the process, on printed newspaper, the operation above described is carried out in the manner described. The news pulp after being reduced in the manner described and then washed in water is

15 found to be of substantially the same color as would be given by a mixture of ground wood and unbleached sulfite. The proportions of ground wood and unbleached sulfite ordinarily used in newspaper stock are 75% of ground wood and 25% of sulfite.

20 The paper which I have made from my recovered book and magazine and newspaper stock is of excellent color, strength and appearance. The recovered fiber, in fact, can be worked back into papers very similar to those from which the fiber is recovered. Newspaper which I have made from my recovered news pulp shows strength which is substantially the same as that of the original 25 paper, from which the fibers are recovered.

30 Experiments which I have conducted have indicated that one pound of book paper will yield about  $12\frac{7}{16}$  ounces of recovered pulp which corresponds to 80% yield or 20% loss, and that one pound of newspaper will yield about 14 ounces of salable pulp or a yield of about 87 $\frac{1}{2}$ % or a loss of 12 $\frac{1}{2}$ %.

35 It will be observed that the lower pipe or draft-tube in which the propellers are mounted is comparatively small in diameter in proportion to the courses of the remainder of the machine. By using this small draft-tube, I secure a great reduction in power and provide a very efficient means of bringing all of the stock into working relation 40 to the over-driven propellers.

45 While my process may be carried out by placing the print paper first in the charging tank to soften it and then feeding it into my de-fibering machine, it will be understood that said process can also be carried out by feeding the paper in dry condition directly to the de-fibering machine. In feeding the paper dry, I prefer to shred the 50 same before feeding it to the de-fibering machine, although it can be roughly torn into pieces and fed in that condition to the de-fibering machine.

55 I have found it advantageous to use more than one propeller in the draft-tube and since the water delivered from the first propeller has a whirling motion, albeit at an angular velocity much less rapid than that of the propeller itself, it is advantageous to have the second propeller of a greater pitch

than the first so as to preserve roughly the same relative angular velocity between the blades and the water.

60 Since the de-fibering and de-inking are co-ordinately important, and in my preferred form take place at the same time, it became necessary to study the conditions most conducive to the latter as well as the former. I have found that de-inking is best accomplished when the amount of water is fairly 70 large relative to the amount of paper. There is a great deal of latitude and some difference depending upon the kind of stock employed and the kind of detergent used, but a fair average working figure is, as previously indicated, 20 parts by weight of water, to 1 part of weight of dry paper. So far as the de-fibering is concerned, the machine will run perfectly well with materially larger proportions of paper but I 75 have found that with concentrations much greater than that named, the whiteness of the pulp becomes progressively less. I have tried smaller degrees of concentration up to 80 several hundred parts of water to one of paper but I find there is a limit beyond 85 which no material advantage in the cleanliness of the product is obtained and the expense of the process is disproportionately increased both in the item of power and of 90 detergent per unit of finished material.

95 In the matter of detergent, assuming that the proper ratio of water to dry paper is employed, I have given a good deal of attention to determining the percentage of dry 100 detergent by weight required for different sorts of paper. It is my present practice to use about 4% on old newspaper, 4 $\frac{1}{2}$ % on magazine and book stock. If a larger 105 amount of water relative to the pulp is used, the amount of detergent must be increased so as to keep the concentration sufficient, but if the amount of water relative to the pulp is diminished, the amount of detergent preferably should not be proportionately diminished since with the relatively insufficient amount of water, the concentration of this material should be somewhat greater in order to get a clean product. I herewith give 110 a formula for detergent which has, all things 115 considered, given the very satisfactory results:—20 pounds of water, 2 pounds of caustic potash, 2 to 3 pounds of tallow or other suitable saponifiable material, 3 pounds of silicate of soda, 2 pounds of 120 chlorid of alumina, 4 pounds of 58% alkali dissolved in 4 pounds of boiling water.

125 Relatively small departures from the preferred formula specified above, produce but very slight changes in the result, but the formula as given may be taken as representing the material which I have found quite satisfactory. It is interesting to note in this connection that the mechanical de-fibering and attrition alone causes the loosening of 130

a considerable percentage of the ink even when no detergent is employed, a circumstance which bears out my theory that the rapid and violent mechanical action in this case is a powerful help to the chemical one.

5 I suppose this to be due to the fact that dried black ink is physically a species of film or incrustation stuck to the paper by the adhesive elements in the ink, but capable of 10 being mechanically loosened by relative motion or separation of the wet matted fibers to which it is stuck, as distinguished, for example, from a dye which enters into and stains the fiber.

15 Black printing ink consists usually of a pigment and a fatty acid or resin or oil as a vehicle, this vehicle carrying the coloring pigment, which in the case of black ink, is usually free carbon. The effect or purpose 20 of the detergent in my process is to saponify the fatty vehicle, which then goes into solution, leaving the particles of pigment free from the vehicle.

25 The ink liberated from the paper or pulp is mixed throughout the pulp and tends to float to the top, carrying with it the carbon which has been freed. The ink residue, together with any filler or mineral matter, or size, starch, etc., which may have been 30 contained in the original paper, are washed from the stock as previously described during the washing operation which follows the de-fibering and de-inking operation.

35 In accordance with the provisions of the patent statutes I have described the principle of operation of my invention together with what I consider the best mode of carrying out the process, but I desire to have it understood that the apparatus is only illustrative and that the invention can be carried out by other means.

40 What is claimed is:

1. A process of de-fibering paper and like materials which consists in immersing the 45 material in a liquid and pulling the fibers of the material apart by subjecting it to opposing forces acting completely below and away from the surface of the liquid, one of which forces is the inertia of the liquid in 50 which the material is suspended.

2. A process for defibering paper and similar materials consisting in immersing the paper in a liquid and feeding this through blades wholly immersed in the 55 liquid and revolving so rapidly that they are able to break down to its component

fibers small pieces of paper fed to them and held relatively against the tendency to revolve at the speed of the blades by their own inertia and that of the liquid in which they 60 are suspended.

3. A process of defibering paper and like materials which consists in immersing the paper in a liquid and feeding this liquid through a screw propeller revolving so rapidly that it is able to defiber small pieces of paper held against the tendency to revolve with the propeller solely by their own inertia and that of the surrounding liquid.

4. A process of defibering paper and like 70 materials which consists in immersing the paper in a liquid and feeding this through a screw propeller immersed in said liquid, revolving so rapidly as to produce a cavity in the liquid effective to promote the de- 75 fibering action.

5. A process of defibering and deinking paper and like materials which consists in immersing the paper in a liquid containing a detergent, and pulling apart the fibers of 80 the paper by an opposition of forces acting completely below and away from the surface of the liquid, one of which forces is the inertia of the paper and the liquid in which it is suspended.

6. A process of de-fibering and de-inking print paper and like material, which consists in softening the paper, then mixing it with a relatively large amount of water containing an emulsifying agent, repeatedly 90 subjecting the mixture to the action of over-driven propelling and agitating elements wholly immersed in the liquid, and subsequently washing the stock.

7. A process of de-fibering and de-inking 95 printed paper, which consists in immersing the paper in a relatively large amount of liquid containing a detergent, circulating the material by means of fast driven propelling agents so that the current of said 100 material on its return passage is subjected to constrictive effect alternatively with subjectation to expanding effect, and in its course passing the liquid through a flaring passage, and finally washing the stock.

105 In testimony that I claim the foregoing as my own, I have hereto affixed my signature in the presence of two witnesses.

OTTO CHARLES WINESTOCK.

Witnesses:

FRANCIS E. GALLAGHER,  
PERRY BARKER.